

# UNITED STATES PATENT OFFICE.

SILAS R. DIVINE, OF LOCH SHELDRAKE, NEW YORK, ASSIGNOR TO THE  
REND ROCK POWDER COMPANY, OF NEW JERSEY.

## EXPLOSIVE COMPOUND.

SPECIFICATION forming part of Letters Patent No. 289,758, dated December 4, 1883.

Application filed July 23, 1883. (No specimens.)

*To all whom it may concern:*

Be it known that I, SILAS R. DIVINE, of Loch Sheldrake, Sullivan county, State of New York, and a citizen of the United States of America, have invented an Improved Explosive Compound, of which the following is a full, clear, and exact specification.

My invention consists in an explosive compound for use chiefly in blasting, composed of a solid ingredient—such as chlorate of potash—and a liquid ingredient consisting of a mixture of nitro-benzole and “dead-oil,” substantially in the proportions and as and for the purposes hereinafter set forth.

15 The object of my present invention is to provide a compound of this character the explosive power or strength of which may be graded or regulated, as desired, and also to provide a compound which may be more economically produced than one in which a fluid nitro compound—such as nitro-benzole alone—constitutes the liquid ingredient.

For economical purposes the desirable proportions in which the nitro-benzole and the dead-oil are mixed to constitute the liquid ingredient are about equal parts of each; and the theoretical proportions in which the solid ingredient of chlorate of potash and the thus constituted liquid ingredient are united to form the explosive are about four or five parts of the solid to one of the liquid, as in this way an explosive of a power or strength substantially equal to one in which nitro-benzole alone is the liquid ingredient is formed at a reduced cost. The exact theoretical proportions need not, however, be strictly adhered to, inasmuch as a preponderance of the nitro-

benzole in the mixture constituting the liquid ingredient will augment the power or strength of the explosive, and a diminution of the nitro-benzole in said mixture will decrease such power or strength; and in the former case it will be found desirable to somewhat decrease the proportion of the chlorate of potash, and in the latter case to somewhat increase the same in the final compound, and the compound be still an effective explosive.

Perchlorate or permanganate of potash may be employed as the solid ingredient, it being understood that the solid ingredient is employed in a crushed or powdered state, and a mixture of other fluid nitro compounds than nitro-benzole and other free fluid and non-volatile hydrocarbons than dead-oil may be employed to constitute the liquid ingredient.

The described ingredients being incapable of explosion by percussion, they can be safely handled and transported, and they can be united by the consumer at the time and place of their desired use by simply permitting the solid to absorb the liquid, or by mixing them in measured proportions in a suitable vessel.

What I claim as my invention, and desire to secure by Letters Patent, is—

The herein-described explosive compound, composed of a solid ingredient—such as chlorate of potash—and a liquid ingredient consisting of a mixture of nitro-benzole and dead-oil, substantially in the proportions and as and for the purposes set forth.

SILAS R. DIVINE.

Witnesses:

A. G. N. VERMILYEA,  
A. S. FITCH.